# EUROPEAN PATENT SPECIFICATION

(11) **EP 3 497 272 B1**
(45) Date of publication and mention of the grant of the patent: **23.12.2020**
(21) Application number: 17761129.0
(22) Date of filing: 02.08.2017
(51) Int. Cl.: D01D 5/088, D01D 10/06, D02G 1/16, D02J 1/08, D01F 6/60, D02G 3/44

(54) **A PROCESS AND AN APPARATUS FOR PRODUCING COARSE COUNT AND TRIDIMENSIONAL CRIMPED MULTIFILAMENT BCF YARNS, YARNS THUS OBTAINED AND APPLICATIONS THEREOF**
EIN VERFAHREN UND EINE VORRICHTUNG ZUR HERSTELLUNG VON GROBEN - UND DREIDIMENSIONAL GEKRÄUSELTEN MULTIFILAMENT-BCF-GARNEN, SO ERHALTENEN GARNEN UND ANWENDUNGEN DAVON
PROCÉDÉ ET APPAREIL POUR LA PRODUCTION DE FILS BCF MULTIFILAMENT FRISÉS ET TRIDIMENSIONNELS FRISÉS GROSSIER, FILS AINSI OBTENUS ET LEURS APPLICATIONS

(30) Priority: 09.08.2016 IT 201600083786
(43) Date of publication of application: 19.06.2019
(73) Proprietor: Bibielle SpA, 12040 Margarita (CN) (IT)
(72) Inventor: BECCARIA, Enrico, 12040 Margarita (CN) (IT); AUDISIO, Riccardo, 12040 Margarita (CN) (IT)
(74) Representative: Lisa, Elisabetta
(86) International application number: PCT/IB2017/054722
(87) International publication number: WO 2018/029577

(56) References cited:
- WO-A1-2015/066689
- US-A- 3 543 358
- US-A- 3 573 133
- US-A- 3 607 610

## Description

### TECHNICAL FIELD

The present invention relates to the field of yarns for non-textile applications and, specifically, to the production and use of multifilament BCF (Bulk Continuous Filament) yarns.

More specifically, the present invention relates to the production and use of coarse count and tridimensional crimped multifilament BCF yarns having controlled chemical-physical and mechanical properties.

More specifically, the present invention relates to a manufacturing process, and the relevant equipment for the production of coarse count and tridimensional crimped multifilament BCF yarns, starting from synthetic materials, in particular polyamide 6.6.

Further, the present invention relates to yarns obtained by the aforesaid process or the aforesaid apparatus both in a wound form and in a cut form.

The present invention finds preferred and beneficial application in non-textile applications, and particularly for the manufacture of carpets for large surfaces.

### STATE OF THE ART

BCF (Bulk Continuous Filament) multifilament yarns, such as are known in the technical field of reference and described, for example, within the U.S. Patent No. US 3 401 516, are continuous yarns composed of many filaments that have been imparted with curling and rippling effects that are typical of natural fibers.

BCF yarns are usually produced by production processes which include spinning by means of molten polymer extrusion, the formation of multiple filaments, drawing and mechanical crimping by air treatment of the multifilament yarns in order to impart to them the aforesaid curling and rippling effects; in general, such traditional production processes allow curling and rippling effects to be obtained only on two axes, namely to achieve two-dimensional crimping of the yarns, which prevents optimal bonding between the baves of the yarns and therefore requires an additional operation known as "interlacing" by interspaced node points in order to hold together the baves of the yarns.

An example of a traditional process for the production of BCF yarns is described in the U.S.

Patent No. US 6 776 943 B2, which envisages starting with polyamide 6 and performing the step of mechanical crimping by a jet of low speed and high temperature air; the BCF yarns produced with this process have an alpha-crystalline content of about 45% and a yarn hank shrinkage of less than about 12.7 mm (0.50 inches); the disadvantages of this solution consist mainly in the fact that the chemical and physical properties cannot be modified insofar as the conditions that determine them cannot be modified and in the fact that the mechanical crimping forces the yard to take a predefined path whereby the shapes obtained in the process (angles and arcs) cannot be varied.

Another example of prior art BCF yarns is disclosed in WO 2015/066689 wherein a coarse count of up to 3,600 denier, i.e. 4,000 decitex, tridimensional crimped multipolymer, multifilament BCF yarn is produced comprising the steps of arranging polyamide 6.6 as a starting material and drying with nitrogen and extruding to obtain filaments. Immediately downstream of the extrusion, the fibers are rapidly quenched in a chimney where cooling air at about 15°C is blown past the filaments through the quench zone. Mechanical treatment follows by drawing and forwarding the filaments into a dual-impingement bulking jet at 200°C (hotair) to produce spun, drawn and crimped bulked continuous filament (BCF).

In addition, the multifilament BCF yarns available generally have uncontrolled chemical-physical (specifically amorphicity/crystallinity degree, basicity and dyeing affinity) and mechanical (specifically elasticity and tenacity) properties.

The bidimensional crimping along with the uncontrolled chemical-physical and mechanical properties of the yarns is the root cause of poor agglomeration problems that occur during the carding of the same, resulting in unevenness of the carded fabric obtained.

Finally, the multifilament BCF yarns currently available have a single filament count of under 40 denier, i.e. 44.44 decitex, and a total count (sum of the counts of the individual filaments) of less than 2,000 decitex.

To achieve workable multifilament BCF yarns in the manufacture of non-textile fabrics it is necessary to reach total counts equal to or greater than 4,000 dtex and this, up until now, has been achieved by means of twisting and cabling operations using multiple yarns; however, these fitting operations, in addition to making the tooling cycle longer and more complicated, also lead to stressing of the yarns and a consequent reduction in the quality thereof.

The need to produce multifilament BCF yarns with tridimensional crimping therefore remains unsatisfied.

Further, the need to control the chemical-physical and mechanical properties of the BCF yarns produced remains unsatisfied.

Finally, the need to produce multifilament BCF yarns with total counts equal to or greater than 4,000 dtex, preferably up to 8,000 dtex, and a count for single-filament up to more than ten times greater than those currently available remains unsatisfied.

In summary, until now, to the knowledge of the Applicant, there are no known solutions that make it possible to avoid the yarn interlacing operations, which overcome the problems of agglomeration that occur during the carding of the same yarns and make it possible to arrange the coarse count multifilament BCF yarns, namely at total counts equal to or greater than 4,000 dtex, preferably up to 8,000 dtex, in order to manufacture technical fabrics without resorting to non-textile twisting and cabling operations using multiple yarns.

Therefore, the Applicant, with the process and the apparatus according to the present invention intends to remedy this deficiency.

### OBJECTS AND SUMMARY OF THE INVENTION

The object of the present invention is to overcome the drawbacks of the known art relating to the production of multifilament BCF yarns.

More precisely, the object of the present invention is to overcome the drawbacks of the known art relating to the production of multifilament BCF yarns in terms of optimal bonding between the baves of the yarns, poor agglomeration and an insufficient count for the manufacture of non-textile technical fabrics.

In particular, the present invention intends to solve the problem of avoiding the yarn interlacing operations, to overcome the single bidimensional crimping and to control the physical-chemical and mechanical properties of the yarns themselves, in order to improve the homogeneity of the BCF yarns obtained and of the subsequent products.

Still in particular, the present invention intends to solve the problem of imparting both high counts for single filament and high total counts of the multifilament BCF yarns for use in the manufacture of non-textile technical fabrics.

These objects are achieved with the process and with the apparatus according to the present invention, advantageously and especially by virtue of cooling in water and of a subsequent non-mechanical treatment with a mixture of air and steam, that make it possible to produce coarse count and tridimensional crimped multifilament BCF yarns having controlled chemical-physical and mechanical properties, in order to improve the agglomeration and homogeneity thereof, to increase the volume thereof and to achieve optimal cohesion between the baves of BCF yarns.

Specifically, the aforesaid objects and other objects and advantages of the invention, as will appear from the following description, are achieved with a process for the production of coarse count and tridimensional crimped multifilament BCF yarns according to claim 1.

Further, the aforesaid objects and other objects and advantages of the invention are achieved with an apparatus for the production of coarse count and tridimensional crimped multifilament BCF yarns according to claim 7.

Further, the aforesaid objects and other objects and advantages of the invention are achieved with coarse count and tridimensional crimped multifilament BCF yarns.

Further, the aforesaid and other objects and advantages of the invention are achieved with a carpet manufactured with coarse count and tridimensional crimped multifilament BCF yarns.

Preferred embodiments and variants of the apparatus for the production of coarse count and tridimensional crimped multifilament BCF yarns, as well as yarns thus obtained and the applications thereof according to the present invention are the subject of the dependent claims; in particular, in preferred and advantageous embodiments, the multifilament BCF yarns according to the present invention may be in a wound form or in a cut form.

Another aspect of the present invention relates to the use of multifilament BCF yarns in non-textile applications, and particularly for the manufacture of carpets for large surfaces.

It is understood that all of the attached claims form an integral part of the present description, and that each of the technical features claimed therein is possibly independent and autonomously usable with respect to other aspects of the invention.

Advantageously, the technical solution according to the present invention makes it possible to:
- increase the count for single filament and the total count of the multifilament BCF yarns, also improving the quality thereof;
- achieve controlled chemical-physical (specifically amorphicity/crystallinity degree, basicity and dyeing affinity) and mechanical (specifically elasticity and toughness) properties of the BCF yarns produced;
- achieve optimum bonding between the baves of the yarns, thus avoiding interlacing operations;
- improve the agglomeration of the yarns, resulting in better product homogeneity;
- simplify the production process, consequently reducing the related costs and consumption of materials; and
- use the BCF yarns produced in the field of non-textile technical fabrics, in particular, for the manufacture of carpets for large surfaces.

Further advantageous features will become more apparent from the following description of preferred but non-exclusive embodiments, provided purely by way of non-limiting examples.

### BRIEF DESCRIPTION OF THE DRAWINGS

The present invention will be described below by means of certain preferred embodiments, given by way of non-limiting examples, with reference to the accompanying drawings. These drawings illustrate different aspects and examples of the present invention and, where appropriate, structures, components, materials and/or similar elements in different figures are indicated by similar reference numbers.
FIG. 1 is a flowchart showing the steps of the process for the production of coarse count and tridimensional crimped multifilament BCF yarns according to the present invention;
FIG. 2 is a schematic representation for the production of coarse count and tridimensional crimped multifilament BCF yarns according to the present invention;
FIG. 3A is a side view schematic representation illustrating the tridimensional crimping of the multifilament BCF yarns according to the present invention;
FIG. 3B is a top view schematic representation illustrating the tridimensional crimping of the multifilament BCF yarns according to the present invention;
FIG. 3C is a tridimensional schematic representation illustrating the tridimensional crimping of the multifilament BCF yarns according to the present invention;
FIG. 4A is a side view schematic representation illustrating the bidimensional crimping of traditional multifilament BCF yarns;
FIG. 4B is a top view schematic representation illustrating the bidimensional crimping of traditional multifilament BCF yarns;
FIG. 4C is a tridimensional schematic representation illustrating the bidimensional crimping of traditional multifilament BCF yarns;
FIG. 5A shows a cross-section of a carpet produced using multifilament BCF yarns according to the present invention;
FIG. 5B shows a plan view of a carpet produced using multifilament BCF yarns according to the present invention;
FIG. 6A shows a cross-section of a carpet produced using traditional BCF yarns; and
FIG. 6B shows a plan view of a carpet produced using tradition BCF yarns.

### DETAILED DESCRIPTION OF THE INVENTION

While the invention is susceptible to various modifications and alternative constructions, certain preferred embodiments are shown in the drawings and will be described in detail below.

In the following description, therefore, the use of "for example", "etc.", "or/or else" means non-exclusive alternatives without limitation, unless otherwise indicated; the use of "also" means "including, but not limited to" unless otherwise indicated; the use of "includes/comprises" means "includes/comprises, but not limited to" unless otherwise indicated.

The process and the apparatus for the production of coarse count and tridimensional crimped multifilament BCF yarns of the present invention, as well as the yarns obtained by this process and/or such apparatus and the applications thereof, are based on the innovative concept of subjecting the extruded polyamide 6.6 filaments to cooling in water and the multifilament BCF yarns obtained to subsequent non-mechanical treatment with a mixture of air and steam, in such a way that the multifilament BCF yarns have controlled chemical-physical and mechanical properties and have a coarse count (both total and for each single filament) as well as tridimensional crimping.

The Inventors have in fact surprisingly and unexpectedly discovered the possibility to achieve a coarse count (both total and for each single filament) by virtue of the cooling in water of extruded polyamide 6.6 filaments and also the tridimensional crimping of the multifilament BCF yarns obtained by virtue of the subsequent non-mechanical treatment with a mixture of air and steam of the latter.

An important feature of said process and apparatus resides in the fact that it is possible to control the chemical-physical (specifically amorphicity/crystallinity degree, basicity and dyeing affinity) and mechanical (specifically elasticity and toughness) properties of the multifilament BCF yarns.

In the present description, the term "filament" or "bave" is meant to indicate the single filament or single bave which, together with a variable number, between 8 and 600, of other filaments or other baves, forms the multifilament BCF yarn; it should be noted that in the present description, the terms "filament" and "bave" are used interchangeably, as synonyms; it should be noted, moreover, that the count of the single filament or single bave, expressed in decitex (d/tex), multiplied by the number of filaments or baves provides the total count, again expressed in decitex (d/tex) of the multifilament BCF thread; each single filament or each single bave can also be expressed, in the literature of the field, in dpf (denier per filament), the conversion between decitex and dpf being known.

In the present description, the term "BCF (Bulk Continuous Filament) yarns" is meant to indicate threads continuously obtained during the spinning step and, thus, differently from yarn threads obtained by means of the process of the spinning of natural or artificial fibers of variable length.

In the present description, the term "multifilament" is meant to indicate a yarn comprising a defined plurality, preferably variable from 8 to 600, of filaments and having a defined dimension expressed in decitex, preferably variable from 13 to 420 decitex.

In the present description, the term "polyamide 6.6" is meant to indicate the material commonly known by the generic name nylon 6.6 having the following chemical formula:

Nylon 6.6 differs from nylon 6 having the following chemical formula:

In the present description, the term "total count" is meant to indicate the sum of the counts of the single filaments that make up the yarn expressed in decitex or denier.

In the present description, the term "total coarse count" is meant to indicate a total count of not less than 4,000 decitex.

In the present description, the term "count for single filament" is meant to indicate the unitary count, expressed in decitex or denier of the single bave or single filament.

In the present description, the term "coarse count for single filament" is meant to indicate a count for single filament of not less than 40 decitex and up to 600 decitex.

In the present description, the term "amorphicity/crystallinity degree" is meant to indicate the ratio within the filament, and specifically of all of the filament, between the amorphous and crystalline areas; it should be noted that the determination of the amorphicity/crystallinity degree is performed using x-ray diffraction.

In the present description, the term "basicity" is intended to indicate the prevalence of basic areas in relation to the acidic areas within the filament; it should be noted that the identification of the basic areas takes place by means of birefringence analysis or else density measurements or else IR spectroscopy; in particular, in this description, the "basicity" is linked to the presence of terminal NH₂ amine groups and, specifically, the basicity increases as the terminal NH₂ amine groups increase (normally the concentration of NH₂ in standard viscosity polyamide 6.6 is around 46 meq/kg, milliequivalents per kg).

In the present description, the term "dyeing affinity" is meant to indicate the ability of the filament to retain the coloring substances within the central core thereof.

In the present description, the term "elasticity" is meant to indicate the ability of the filament to deform under the action of external forces applied thereto and to regain the initial shape thereof when the applied external forces cease.

In the present description, the term "tenacity" is meant to indicate the ability of the filament to absorb an amount of energy per unit of volume without breaking; in order to measure the "tenacity" the splitting strength (cN) can be used in relation to the initial filament count (tex or decitex).

In the present description, the term "agglomeration" is meant to indicate the ability to bond between individual filaments or cut portions of BCF yarns in order to achieve a non-woven fabric, commonly called "web"; it should be noted that the ability to bond between the filaments takes place when the filaments themselves remain naturally linked together, without the need for further tooling or the use of additives.

In the present description, the term "cohesion" is meant to indicate the predisposition of the BCF yarn filaments or cut portions to interlace between them evenly and without the aid of further tooling or the use of additives.

In the present description, the term "homogeneity" is meant to indicate the regularity of weight and thickness due to the bonding.

In the present description, the term "crimping" is meant to indicate the process in order to impart to the filaments or cut portions of BCF yarns the nonlinear wrinkling curves that are exemplary of natural fibers.

In the present description, the term "wrinkling" is meant to indicate the particular curling and rippling imparted to the filaments or cut portions of BCF yarns with the aforementioned crimping process.

In the present description, the term "non-textile technical fabrics" is meant to indicate products other than those that are textile; non-textile technical fabrics are differentiated by the requirement of having to tolerate much higher mechanical stresses, starting from 100% higher.

With reference to Fig. 1, the process for producing coarse count and tridimensional crimped multifilament BCF yarns, comprises the following steps:
- arranging polyamide 6.6 as starting material (step 100);
- drying said polyamide 6.6 with nitrogen (step 101);
- extruding said polyamide 6.6, thus obtaining filaments (6a) (step 102);
- immediately downstream of the extrusion, cooling in water the filaments 6a obtained in the previous step 102 at a predetermined temperature ranging between 17°C and 50°C and for a predetermined time ranging between 0.5 seconds and 0.8 seconds, thus obtaining coarse count multifilament BCF yarns (6b) (step 103);- subjecting to a non-mechanical treatment with a mixture of air and steam said coarse count multifilament BCF yarns (6b) obtained in the previous step 103, wherein the amounts of air and steam are in a predetermined ratio between them ranging between 30:70 by volume and 60:40 by volume, thus obtaining coarse count and tridimensional crimped multifilament BCF yarns 6c (step 104). Optionally, the process according to the present invention may also include the following step:
   - between step 101 and step 102, adding coloring substances.

According to the present invention, the optional dyeing operation is performed en masse, specifically in adding bulk coloring substances to the starting material, for example as granules or powder; preferably the coloring substances are natural and artificial pigments; more preferably, the coloring substances are a balanced mixture of natural and artificial pigments, because natural pigments are brighter and lively but tend to suffer migration in water, while the artificial pigments are less lively but do not migrate and therefore are technically superior.

According to step 100 of this invention, polyamide 6.6 is used as the starting material; in particular, the polyamide 6.6 used is in the form of granules or "chips," with an average particle size in the order of 2 mm x 2 mm x 3 mm.

As mentioned above, the polyamide 6.6 used in the present invention has the chemical formula reported above and preferably has a fusion point equal to 260°C and a specific weight equal to 1.15 g/cm³.

According to the subsequent step 101 of the present invention, the polyamide 6.6 is dried with nitrogen.

This operation is performed within drying towers, for an average duration of 10 hours at an average temperature of 82°C.

The nitrogen used is preferably 90% pure; the flow of nitrogen is made to flow with an average flow rate of 20 kg/h.

The dried polyamide 6.6 has a residual moisture content of less than 700 p.p.m. (parts per million), or less than 0.07% by weight of polyamide 6.6.

According to the subsequent step 102 of the present invention, the dried polyamide 6.6 is extruded, thus obtaining the filaments 6a.

The extrusion is performed in a conventional spinneret and will therefore not be described in detail.

The filaments 6a of polyamide 6.6 obtained by means of extrusion in the previous step 102 are then, immediately downstream of the extrusion, cooled in water at a temperature and for a predetermined period of time, according to step 103 of the present invention.

The cooling in water takes place in a tank placed at a distance equal to or less than 5 mm from the exit from an extruder, wherein the temperature of the cooling water ranges between 17°C and 50°C, preferably it is equal to 35°C, and wherein the cooling time ranges between 0.5 seconds and 0.8 seconds, preferably it is equal to 0.6 seconds.

Further, the cooling in water takes place at a speed ranging from 5,800 mm/second and 8,300 mm/second, preferably equal to 6,000 mm/second.

As anticipated, the Inventors have surprisingly and unexpectedly discovered that the cooling in water of extruded polyamide 6.6 filaments 6a under the conditions indicated above, and specifically at a high speed, makes it possible to achieve coarse count filaments for each single filament and corresponding total coarse count multifilament BCF yarns 6b.

In particular, the filaments obtained by the process according to the invention include a count for each single filament of up to 420 decitex, and the corresponding coarse count multifilament BCF yarns 6b have a total count equal to or greater than 4,000 decitex, preferably up to 8,000 dtex.

By way of comparison it is reported that the filaments obtained by traditional processes have a count for each single filament up to 44 decitex, and the corresponding multifilament BCF yarns have a total count up to 2,000 decitex.

Further, the cooling in water according to step 103 of the present invention makes it possible to control the chemical-physical and mechanical properties of the multifilament BCF yarns.

Specifically, the process according to the present invention makes it possible to control the amorphicity/crystallinity degree, the basicity and dyeing affinity as chemical-physical properties, and the elasticity and tenacity as mechanical properties.

The Inventors believe that controlling the speed of the cooling in water of the individual extruded filaments makes it possible to control their percentage content of amorphous zones, upon which depend the amorphicity/crystallinity degree, the basicity and the dyeing affinity; in particular, the higher the cooling speed, the more, within individual filaments, the amorphous zones prevail with respect to the crystalline zones; a filament with a higher degree of amorphicity means that few amide groups are engaged in the formation of hydrogen bridges and this, consequently, results in increased basicity and in the improved dyeing affinity of the individual filaments and of the corresponding multifilament BCF yarns. The Inventors believe that also the uniformity of the cooling in water, by virtue of the increased heat transfer efficiency between the single filaments and the water itself, contributes to the improvement of the chemical-physical and mechanical properties thereof.

In more detail the amorphicity/crystallinity degree, as a function of the cooling/glass transition speed, is controllable through the cooling water temperature; in traditional spinning processes the crystalline composition prevails insofar as the glass translation is slower (approximately five times slower) and the molecules have time to orient themselves in the same direction, increasing the degree of crystallinity.

According to the Inventors, the control of the amorphicity/crystallinity levels is due to the polyamide 6.6 solidification speed.

As mentioned above, the basicity is a function of the amorphicity/crystallinity degree and therefore by X-ray spectrometry (birefringence), density, FTIR (infrared spectroscopy) and DSC (Differential Scanning Calorimetry) measurements, it can be stated that the multifilament BCF yarns according to the present invention are more basic than traditional BCF yarns.

As mentioned above, the dyeing affinity depends also upon the percentage of amorphous zones in the filaments, and therefore the multifilament BCF yarns according to the present invention have better dyeing affinity than traditional BCF yarns; it should be noted that it is the amorphous areas that receive the coloring and, therefore, the colors of the multifilament BCF yarns according to the present invention remain more vivid, natural and shiny.

According to the Inventors, the control of the dyeing affinity is due to the control over the creation of the amorphous zones.

The elasticity also depends upon the amorphous/crystalline properties of the yarn and, consequently, better elasticity corresponds to a greater presence of amorphous zones; it should be noted that the elasticity is expressed as a percentage of the original length of the sample.

According to the Inventors, the control over the elasticity is due to the glass transition temperature and therefore of the orientation and mobility of the molecules within the filament that enable the filament itself to be drawn in order to achieve the tenacity, but at the same time to not lose the elasticity.

The relationship between elasticity and tenacity is narrow and proportional; an elastic thread will not be tenacious because it has undergone little stretching, namely an extension of less than 100% of the original length, while a tenacious thread is not elastic because it has undergone significant stretching, namely an extension greater than 150% of the original length.

The tenacity depends upon the amount of strength that must be exercised in order to elongate the filament; according to the Inventors, the control over the tenacity is mainly due to the cooling in water conditions according to the step 103, as mentioned above, and to the drawing conditions.

The coarse count of the yarns makes it possible to avoid interlacing operations and those of twisting and cabling of multiple yarns, in such a way as to achieve higher-quality products and also to simplify and speed up the production process.

The coarse count multifilament BCF yarns obtained in the previous step 103 are, subsequently, subjected to non-mechanical treatment with a mixture of air and steam, wherein the amounts of air and steam are in a predetermined ratio between them, according to step 104 of the present invention.

It is to be pointed out here that "non-mechanical treatment" is meant to indicate a treatment that, unlike traditional mechanical treatments, is not accomplished by contact with the crimping device; the non-mechanical treatment according to the present invention instead envisages the passage of the multifilament BCF yarns within a device containing a mixture of air and steam, without the exercising of any mechanical action, and therefore contact, of the device upon the multifilament BCF yarns; in summary, the term "non-mechanical treatment" is used, in this description, as a synonym for "treatment without contact with the crimping device".

As anticipated, the Inventors have surprisingly and unexpectedly discovered that the non-mechanical treatment with a mixture of air and steam of coarse count polyamide 6.6 multifilament BCF yarns under the conditions indicated above makes it possible to obtain tridimensional crimped multifilament BCF yarns.

The amounts of air and steam are in a ratio ranging between 30:70 and 60:40 by volume.

With reference to Figs. 3A-3C and 4A-4C, respectively visible are the tridimensional crimping of the multifilament BCF yarns according to the present invention in comparison to the bidimensional crimping of traditional BCF yarns; in particular, Figs. 3A and 4A are side views, Figs. 3B and 4B are views from above and Figs. 3C and 4C are tridimensional views.

As can be seen, the multifilament BCF yarns according to the present invention, by virtue of the tridimensional crimping, have profiles that are curvilinear and variously oriented in space; conversely, the traditional multifilament BCF yarns, due to the bidimensional crimping, have cracked profiles that are oriented along only two directions in space.

The tridimensional crimping of the yarns makes it possible to obtain optimal bonding between the baves of the yarns and to improve the agglomeration thereof, in order to obtain products of better quality.

With reference to Fig. 2, the apparatus 1 for the production of coarse count and tridimensional crimped multifilament BCF yarns, that makes up an independent and autonomously usable aspect in relation to the other aspects of the invention, comprises:
- a feed hopper 2 for polyamide 6.6;
- a drying room 3 for drying said polyamide 6.6 with nitrogen;
- an extruder 4 for extruding said polyamide 6.6, thus obtaining filaments 6a;
- immediately downstream of the extruder 4, a tank 5 for cooling in water said filaments 6a, thus obtaining coarse count multifilament BCF yarns 6b;
- a device 7 comprising a compartment 8 and a tube 9 placed inside said compartment 8, said compartment 8 being suitable to house a mixture of air and steam and said tube 9 being suitable to host said coarse count multifilament BCF yarns 6b previously obtained, thus obtaining coarse count and tridimensional crimped multifilament BCF yarns 6c.

The feed hopper 2, the drying chamber 3 and the extruder 4 are of a conventional type and, therefore, will not be described in detail.

The extruder 4, however, may be appropriately modified in such a way that the filaments assume different sections such as, for example, in the shape of a "delta", trilobal, mixed polygonal and/or curvilinear, and so on, according to the specific requirement.

The tank 5 for cooling the filaments 6a in water, placed immediately downstream of the extruder 4 envisages that the path of the filaments 6a be modifiable both as to the length thereof and the depth and is preferably manufactured from stainless steel; preferably, said tank 5 contains osmotic water, preferably in an amount of 500 liters; it is evident that the amount of water can be modified according to specific requirements.

In more detail and according to a preferred embodiment of the invention (not shown), in order to modify the path of the filaments 6a in length and depth, within said tank 5 plasma coated stainless steel rollers are positioned, in order to promote the slipping of the filaments 6a; said rollers, preferably in a number equal to four, are mounted on a single plunging arm which, depending upon the assigned inclination which is adjustable by suitable means, increases or decreases the depth thereof in water, from surface free up to being in contact with the bottom of the tank, and lengthens or shortens the path of the filaments 6a up to ± 30% and, consequently, the period of time that the same remain in water; as mentioned above, the pitch of the plunging arm is assigned according to the specific requirements and is appropriately adjusted between five preset positions by as many mechanical end-of-travel stops of the same arm; the pitch can vary between 30° and 60° with respect to the direction of entry into the tank of the filaments 6a.

The tank 5 for cooling the filaments 6a in water is preferably placed at a distance equal to or shorter than 5 mm from the exit from the extruder 4, in order to obtain coarse count multifilament BCF yarns 6b.

The device 7, which comprises a compartment 8 and a tube 9 placed inside said compartment 8, is of a variable size from 0.6 to 5 mm depending upon the bundle of threads to be housed, it is perforated in order to ensure controlled roughness and is preferably manufactured from stainless steel; this configuration of the device 7 makes it possible to obtain coarse count and tridimensional crimped multifilament BCF yarns 6c.

The apparatus 1 may further comprise means 10 (not shown) for wrapping said coarse count and tridimensional crimped multifilament BCF yarns 6c; these means 10 for wrapping the yarns are known and are therefore not discussed in detail.

As an alternative to the aforementioned configuration, the apparatus 1 may further comprise means 20 (not shown) for cutting said coarse count and tridimensional crimped multifilament BCF yarns 6c; these means 20 for cutting the yarns are known and are therefore not discussed in detail.

The multifilament BCF yarns obtained by the process and/or through the device according to the present invention, make it possible, therefore, to attain advantageous features and properties.

In particular, the coarse count and tridimensional crimped multifilament BCF yarns obtained through the process disclosed above and/or with the apparatus described above, which constitute an aspect that is independent and autonomously usable with respect to other aspects of the invention, having a total count equal to or higher than 4,000 decitex, preferably up to 8,000 dtex, with each filament having a count up to 420 decitex, and having controlled chemical-physical and mechanical properties, in particular the amorphicity/crystallinity degree ranges between 70/30% and 50/50%, preferably it is equal to 60/40%, the basicity ranges between 4 French degrees and 10 French degrees, preferably it is equal to 7 French degrees, the dyeing affinity ranges between 80% and 95%, preferably it is higher than 90%, the elasticity ranges between 30% and 100%, preferably it ranges between 40% and 70%, more preferably it is equal to 60% and the tenacity ranges between 15 cNW/tex and 50 cNW/tex, preferably it is equal to 30 cNW/tex. It should be noted that the use of French degrees to measure basicity is known in the reference field of the invention.

The coarse count and tridimensional crimped multifilament BCF yarns according to the present invention may be in a wound form or in a cut form.

As mentioned above, the coarse count and tridimensional crimped multifilament BCF yarns according to the present invention are particularly suitable for non-textile applications; preferably and advantageously, the coarse count and tridimensional crimped multifilament BCF yarns according to the present invention are employed in the manufacture of carpets for large surfaces.

It therefore, finally, constitutes an aspect that is independent and autonomously usable with respect to the other aspects of the invention 50, manufactured with coarse count and tridimensional crimped multifilament BCF yarns 6c.

With reference to Figs. 5A and 5B, it is observed that the carpet 50 according to the present invention is produced with multifilament BCF yarns according to the present invention, which does not need to be further treated with twisting or other assembly processes; by way of comparison, in Figs. 6A and 6B, a carpet 50' produced with traditional BCF yarns is visible; in particular, Figs. 5A and 6A are cross-sections and Figs. 5B and 6B are plan views.

As can be seen, the carpet 50 according to the present invention, by virtue of the use of coarse count and tridimensional crimped multifilament BCF yarns 6c, has a flat structure; conversely, the carpet 50' produced using traditional coarse count and bidimensional crimped multifilament BCF yarns, has a twisted structure.

The carpet 50 according to the present invention is manufactured using wrapped multifilament BCF yarns.

The carpet 50 according to the present invention has advantages such as the absence of unsightly "pills", due to the fact that the thread used is not twisted, of durable color, has stain-resistant properties and is resistant to wear and abrasion; these properties are demonstrated by the following tests.

As can be deduced from the above, the innovative technical solution described here has the following advantageous features:
- the increase in the count for single filament and of the total count of the multifilament BCF yarns, also improving the quality thereof;
- the achieving of controlled chemical-physical (specifically amorphicity/crystallinity degree, basicity and dyeing affinity) and mechanical (specifically elasticity and toughness) properties of the BCF yarns produced;
- the achieving of optimum bonding between the baves of the yarns, thus avoiding interlacing operations;
- the improving of the agglomeration of the yarns, resulting in better product homogeneity;
- the simplification of the production process and consequent reduction of the associated costs and consumption of materials; and
- the possibility of using the BCF yarns produced in the field of non-textile technical fabrics, in particular, for the manufacture of carpets for large surfaces.

From the description above it is evident, therefore, how the technical solution according to the present invention, in the different aspects thereof, would achieve the objects proposed.

## Claims

1. A process for producing coarse count and tridimensional crimped multifilament BCF yarns, comprising the following steps:
- arranging polyamide 6.6 as starting material (step 100);
- drying said polyamide 6.6 with nitrogen (step 101);
- extruding said polyamide 6.6, thus obtaining filaments (6a) (step 102);
- immediately downstream the extrusion, cooling in water the filaments (6a) obtained in the previous step 102 at a predetermined temperature ranging between 17°C and 50°C and for a predetermined time ranging between 0.5 seconds and 0.8 seconds, thus obtaining coarse count multifilament BCF yarns (6b) (step 103);
- subjecting to a non-mechanical treatment with a mixture of air and steam said coarse count multifilament BCF yarns (6b) obtained in the previous step 103, wherein the amounts of air and steam are in a predetermined ratio between them ranging between 30:70 by volume and 60:40 by volume, thus obtaining coarse count and tridimensional crimped multifilament BCF yarns (6c) (step 104).

2. A process according to claim 1, wherein the cooling in water takes place in a tank placed at a distance equal to or lower than 5 mm from the exit from an extruder, at a speed ranging between 5,800 mm/second and 8,300 mm/second, wherein the temperature of the cooling water is equal to 35°C, and wherein the cooling time is equal to 0.6 seconds.

3. A process according to claim 2, wherein the cooling in water takes place at a speed equal to 6,000 mm/second.

4. A process according to claim 1 or 2 or 3, wherein the amounts of air and steam are in a ratio 45:55 by volume.

5. A process according to any of the preceding claims, wherein the obtained coarse count multifilament BCF yarns have a total count equal to or higher than 4,000 decitex and wherein each filament has a count up to 420 decitex.

6. A process according to any of the preceding claims, further comprising the following step:
- between step 101 and step 102, adding coloring substances.

7. An apparatus (1) for producing coarse count and tridimensional crimped multifilament BCF yarns using polyamide 6.6 as starting material, comprising:
- a feed hopper (2) for feeding said polyamide 6.6;
- a drying tower (3) for drying said polyamide 6.6 with nitrogen;
- an extruder (4) for extruding said polyamide 6.6, thus obtaining filaments (6a);
- immediately downstream the extruder (4), at a distance equal to or lower than 5 mm from the exit from the extruder (4), a tank (5) for cooling in water said filaments (6a), thus obtaining coarse count multifilament BCF yarns (6b);
- a device (7) comprising a compartment (8) and a tube (9) placed inside said compartment (8), said compartment (8) being suitable to house a mixture of air and steam and said tube (9) being suitable to host said coarse count multifilament BCF yarns (6b) previously obtained, thus obtaining coarse count and tridimensional crimped multifilament BCF yarns (6c).

8. An apparatus (1) according to claim 7, further comprising:
- means (10) for winding said coarse count and tridimensional crimped multifilament BCF yarns (6c).

9. An apparatus (1) according to claim 7, further comprising:
- means (20) for cutting said coarse count and tridimensional crimped multifilament BCF yarns (6c).

## Patentansprüche

1. Verfahren zur Herstellung von groben dreidimensionalen gewellten BCF Mehrfilament-Garnen, umfassend folgende Schritte:
- ein Polyamid 6.6 als Ausgangsmaterial einsetzen (Schritt 100);
- das Polyamid 6.6 mit Stickstoff trocknen (Schritt 101);
- das Polyamid 6.6 extrudieren, wodurch Filamente (6a) erhalten werden (Schritt 102);
- unmittelbar nach der Extrusion, die im vorherigen Schritt 102 erhaltenen Filamente (6a) in Wasser bis auf eine vorbestimmte Temperatur zwischen 17°C und 50°C und für eine vorbestimmte Zeit zwischen 0,5 Sekunden und 0,8 Sekunden abkühlen, wodurch grobe BCF Mehrfilament-Garne (6b) erhalten werden (Schritt 103);
- die im vorherigen Schritt 103 erhaltenen BCF groben Mehrfilament-Garne (6b) einer nichtmechanischen Behandlung mit einem Gemisch aus Luft und Dampf unterziehen, wobei die Luft- und Dampfmengen in einem vorbestimmten Volumen-Verhältnis von 30:70 und 60:40 stehen, wodurch grobe dreidimensionale gewellte BCF-Mehrfilament-Garne (6c) erhalten werden (Schritt 104).

2. Verfahren nach Anspruch 1, wobei das Abkühlen in Wasser in einem Tank in einem Abstand von höchstens 5 mm vom Auslass eines Extruders mit einer Geschwindigkeit zwischen 5800 mm/s und 8300 mm/s erfolgt, wobei die Kühlwassertemperatur 35°C beträgt und die Kühlungszeit 0,6 Sekunden beträgt.

3. Verfahren nach Anspruch 2, wobei das Abkühlen in Wasser mit einer Geschwindigkeit von 6000 mm/s erfolgt.

4. Verfahren nach Anspruch 1 oder 2 oder 3, wobei die Luft- und Dampfmengen sich in einem Volumenverhältnis von 45:55 befinden.

5. Verfahren nach einem der vorhergehenden Ansprüche, wobei dem die groben BCF Mehrfilament-Garne eine Gesamtanzahl von 4000 Decitex oder mehr aufweisen und wobei jedes Filament eine maximale Anzahl von 420 Decitex aufweist.

6. Verfahren nach einem der vorhergehenden Ansprüche, ferner umfassend folgenden Schritt:
- zwischen Schritt 101 und Schritte 102 Farbstoffe hinzufügen.

7. Vorrichtung (1) zur Herstellung von groben dreidimensionalen gewellten BCF Mehrfilament-Garnen unter Verwendung von Polyamid 6.6 als Ausgangsmaterial, umfassend:
- einen Zuführtrichter (2) zum Zuführen des Polyamids 6.6;
- einen Trockenturm (3) zum Trocknen des Polyamids 6.6 mit Stickstoff;
- einen Extruder (4) zum Extrudieren des Polyamids 6.6, wodurch Filamente (6a) erhalten werden;
- unmittelbar stromabwärts des Extruders (4) in einem Abstand von 5 mm oder weniger vom Ausgang des Extruders (4), einen Tank (5) zum Abkühlen der Filamente (6a) in Wasser, wodurch grobe BCF Mehrfilament-Garne (6b) erhalten werden;
- eine Vorrichtung (7), die ein Fach (8) und ein Rohr (9) umfasst, die sich in dem Fach (8) befindet, wobei das Fach (8) zur Aufnahme eines Gemisches aus Luft und Dampf und das Rohrs (9) ist geeignet, um die zuvor erhaltenen groben BCF Mehrfilament-Garne (6b) unterzubringen, wodurch grobe dreidimensionale gewellte BCF Mehrfilament-Garne (6c) erhalten werden.

8. Vorrichtung (1) nach Anspruch 7, ferner umfassend:
- Mittel (10) zum Aufwickeln der groben dreidimensionalen gewellten BCF Mehrfilament-Garne (6c).

9. Vorrichtung (1) nach Anspruch 7, ferner umfassend:
- Mittel (20) zum Schneiden der groben dreidimensionalen gewellten BCF Mehrfilament-Garne (6c).

## Revendications

1. Procédé de production de fils multi-filaments BCF ondulés épais et tridimensionnels, comprenant les opérations suivantes:
- placer un polyamide 6.6 comme matière de départ (opération 100);
- sécher ledit polyamide 6.6 avec de l'azote (opération 101);
- extruder ledit polyamide 6.6, obtenant ainsi des filaments (6a) (opération 102);
- immédiatement en aval de l'extrusion, refroidir les filaments (6a) obtenus lors de l'opération précédente 102 dans l'eau à une température prédéterminée comprise entre 17°C et 50°C et pendant une durée prédéterminée comprise entre 0,5 seconds et 0,8 seconds, obtenant ainsi des fils multi-filament BCF épais (opération 103);
- soumettre lesdits fils multi-filaments épais (6b) obtenus lors de l'opération précédente 103 à un traitement non mécanique avec un mélange d'air et de vapeur, dans lequel les quantités d'air et de vapeur sont comprises dans un rapport prédéterminé entre elles 30:70 en volume et 60:40 en volume, obtenant ainsi des filaments multi-filaments BCF tridimensionnels épais et ondulés (6c) (opération 104) .

2. Procédé selon la revendication 1, dans lequel le refroidissement dans l'eau a lieu dans une cuve située à une distance égale ou inférieure à 5 mm de la sortie d'une extrudeuse, avec une vitesse comprise entre 5800 mm/s et 8300 mm/s, dans laquelle la température de l'eau de refroidissement est égale à 35°C, et dans laquelle le temps de refroidissement est égal à 0,6 secondes.

3. Procédé selon la revendication 2, dans lequel le refroidissement dans l'eau a lieu avec une vitesse égale à 6000 mm/s.

4. Procédé selon les revendications 1 ou 2 ou 3, dans lequel les quantités d'air et de vapeur sont comprises dans un rapport de 45:55 en volume.

5. Procédé selon l'une des revendications précédentes, dans lequel les fils multi-filaments BCF épais obtenus ont un titre total égal ou supérieur à 4000 décitex et dans lequel chaque filament a un titre maximum de 420 décitex.

6. Procédé selon l'une des revendications précédentes, comprenant en outre l'opération suivante:
- entre l'opération 101 et l'opération 102, ajouter des matières colorantes.

7. Dispositif (1) de production de fils multi-filaments BCF tridimensionnels ondulés et épais en utilisant du polyamide 6.6 comme matière de départ, comprenant:
- une trémie d'alimentation (2) pour alimenter ledit polyamide 6.6;
- une tour de séchage (3) pour sécher ledit polyamide 6.6 avec de l'azote;
- une extrudeuse (4) pour extruder ledit polyamide 6.6, en obtenant ainsi des filaments (6a);
- immédiatement en aval de l'extrudeuse (4), à une distance égale ou inférieure à 5 mm de la sortie de l'extrudeuse (4), une cuve (5) pour refroidir lesdits filaments (6a) dans l'eau, en obtenant ainsi des fils multi-filament épais (6b);
- un dispositif (7) comprenant un compartiment (8) et un tube (9) situé à l'intérieur dudit compartiment (8), ledit compartiment (8) étant apte à loger un mélange d'air et de vapeur et ledit tube (9) étant apte à loger lesdits fils multi-filament BCF épais (6b) précédemment obtenus, en obtenant ainsi des fils multi-filaments ondulés épais et tridimensionnels (6c).

8. Appareil (1) selon la revendication 7, comprenant en outre:
- des moyens (10) pour enrouler lesdits fils multi-filaments BCF ondulés épais et tridimensionnels (6c).

9. Appareil (1) selon la revendication 7, comprenant en outre:
- des moyens (20) pour couper lesdits fils multi-filaments BCF ondulés épais et tridimensionnels (6c).
